

## UNITED STATES PATENT OFFICE

2,048,796

## TREATMENT OF TEXTILE MATERIALS

Ernest William Kirk and George Holland Ellis,  
Spondon, near Derby, England, assignors to  
Celanese Corporation of America, a corporation  
of Delaware

No Drawing. Application May 26, 1934, Serial  
No. 727,736. In Great Britain June 9, 1933

1 Claim. (Cl. 8—5)

This invention relates to the colouration of textile materials and more particularly to the colouration of textile materials by methods involving the formation of difficultly soluble azo dyes thereon from suitable components.

The formation of difficultly soluble azo dyestuffs on textile materials from diazo compounds and phenolic coupling components, especially the arylamides of 2:3-oxynaphthoic acid, constitutes a very valuable method for colouring the said materials. As usually practised, the material is impregnated with the coupling component and the latter then caused to couple with a diazo compound. In the case of cotton, regenerated cellulose, or other cellulose material, it is the usual practice to impregnate the material with the coupling component and then to treat with a solution of a diazo compound. In the case of some materials, however, and particularly in the case of cellulose acetate or other cellulose ester or ether materials, it is often found more convenient to diazotize the diazo component on the material and thereafter to apply the coupling component or, alternatively, to apply both the diazo component and the coupling component to the material either together or separately and thereafter subject the material to treatment to effect diazotization and coupling. In the case of cellulosic materials, for example cotton, the impregnation of the material with the coupling component is easily effected from alkaline solutions, which may readily be obtained with the aid of several equivalents of caustic alkali to each equivalent of coupling component. From such solutions the components are readily absorbed by the cotton, which is not damaged by the alkali, even when the latter is present in relatively high concentrations. In the case of cellulose ester materials, however, if caustic alkali is used in proportions sufficient to ensure in all cases the solution of the coupling component, there is grave danger of saponifying the ester under the conditions of temperature, concentration, etc., such as are usually employed in dyeing operations of the character in question. It is therefore necessary to restrict the proportion of alkali in the impregnating medium if saponification is to be avoided.

These considerations apply generally to coupling components which require alkali to effect solution in water, for example aromatic hydroxy compounds, e. g. the above-mentioned arylamides of 2:3-oxynaphthoic acid and also coupling compounds containing the grouping

—CH<sub>2</sub>CO—,

e. g. arylamides of aceto-acetic acid. All these coupling components which, at least in the enol

form, containing a hydroxy group, are herein-after referred to as enolic coupling components.

We have observed that when applying enolic coupling components to cellulose ester materials from baths made with such small proportions of alkalies as to avoid material saponification of the ester, small variations in the alkalinity of the bath have a very marked effect upon the affinity of the coupling component for the ester. In consequence, it is advantageous to control the degree of alkalinity within very narrow limits to obtain uniform and consistent results, and in particular if the full colour value of the coupling component is to be utilized. This is particularly the case with coupling components such as the arylamides of 2:3-oxynaphthoic acids, which are not readily maintained in solution, colloidal or otherwise, except under rather strong alkaline conditions.

We have now found that in the impregnation of cellulose ester materials with enolic coupling components from alkaline media, the addition of a sugar to the alkaline solutions of the coupling components is of great benefit. The sugar, we have found, enables a greater proportion of alkali to be employed in preparing the impregnation medium than is otherwise permissible, if material saponification of the ester is to be avoided. In particular the addition of the sugar enables the proportion of alkali employed to be that most advantageous from the point of view of causing the absorption of the coupling component to be as uniform and complete as possible, while yet avoiding saponification.

The new process of impregnating cellulose ester materials with an enolic coupling component consists essentially in applying to the material a preparation containing the constituents of a composition obtainable by adding a sugar to an alkaline solution of the enolic coupling component. Preparations containing the said constituents are included in the scope of the invention.

By working according to the new process, it is thus possible to secure even colouration and effective utilization of the colour value of the coupling component, while at the same time avoiding a saponification of the material. Moreover, in the presence of the sugar the proportion of alkali requisite to secure these results is by no means critical, a very great advantage in practice.

The utility of the new process is not, however, restricted to the colouration of cellulose ester materials, as it may be applied to colouring of other materials, especially such as absorb enolic coupling components to best advantage from media prepared with greater proportions of alkali than can be otherwise tolerated if damage of the materials is to be avoided.

- The beneficial action of the sugar is probably due to its buffering action, that is its tendency to render the alkalinity of aqueous media no longer completely dependent on the proportion of alkali employed. We have indeed found that the sugar may be replaced by other buffering agents. As examples of such other agents may be mentioned polyhydric alcohols, for example mannitol and also substances of weakly acidic character, for example the amino acids, especially the aliphatic amino acids, and the di- or poly-peptides in which two or more amino acid residues are united, as for example in glycyl-glycine. Suitable amino acids or di- or poly-peptides are, for example, those readily obtainable by the acid or alkaline hydrolysis of proteins. If desired, crude hydrolysis products may be employed, for example the crude products obtainable by hydrolyzing wool or like protein material with aqueous alkali. Again weak inorganic acids may be employed, for example boric acid. Weak di- or poly-basic acids are advantageous. There may be employed in general neutral to weakly acid substances which are capable of forming salts with alkalies. Extremely satisfactory results may, however, be obtained with sugars, and it is preferred to use these bodies. Various sugars may be used, for example cane sugar or other dioses or polyoses. Particularly good results may, however, be obtained by the use of reducing sugars, for example dextrose, laevulose, galactose, or other monoses, or crude products containing these reducing sugars, for example the mixture of glucose and laevulose obtainable by hydrolyzing cane sugar or a crude sugar-containing mixture obtainable by hydrolysis of wood.
- The reducing sugars are of especially great advantage when it is required to apply the diazo component simultaneously with the coupling component, which method, as explained above, is frequently practiced in connection with the colouration of cellulose ester materials. The reducing sugar has the very valuable property of restricting the oxidation of the diazo component, a matter of particular importance when the diazo component is a body which is comparatively readily oxidized, for example amino-diphenylamine derivatives, e. g. 4:4'-diamino-diphenylamine. The latter base, in particular, is readily oxidized by the air and in the absence of any precaution to prevent oxidation may become so seriously oxidized when dyeing on a winch machine or other machine in which the air has free access to the materials, as to render the resulting dyes substantially useless. If desired, the sugar or other buffering agent may be employed in conjunction with a reducing agent and as an example of such a reducing agent, mention may be made of phenyl hydrazine sulphonic acid.
- The proportion of alkali employed in preparing the impregnation liquors containing the enolic coupling components may vary within comparatively wide limits, for as explained above, the presence of the sugar or other buffering agent tends to render the alkalinity of the bath no longer completely dependent on the proportion of alkali employed. For example, caustic alkali sufficient for complete salt formation with the coupling component may be employed. Particularly good results have, however, been obtained by the employment of caustic alkali in the proportion of about two equivalents per equivalent of a mono-2:3-oxy-naphthoic aromatic amine, for example 2:3-oxy-naphthoic acid anilide. In the case of coupling components containing two or

more oxy-naphthoic acid amide groups, proportionately greater quantities of alkali should be employed. Similar considerations apply in connection with other coupling components, that is to say the quantity of alkali may advantageously be about that required for complete salt formation with the coupling component. 5

The proportion of sugar or other buffering agent employed is not critical but should preferably be such as to contain a sufficient proportion 10 of hydroxy, carboxylic or other groups capable of forming salts with alkali metals, to combine with the alkali employed. In practice very good results have been obtained by the employment of glucose or other reducing sugar in about twice 15 the weight of the caustic alkali used for effecting solution of the coupling component.

For application to textile materials, the solutions of the coupling components may be in the form of either freely fluid liquids for application 20 by bath methods, or in the form of thickened preparations suitable for application by padding, printing or other method of mechanical impregnation. The impregnation baths or padding or printing liquors are very readily prepared simply 25 by dissolving the coupling component with the requisite amount of caustic alkali, for example caustic soda, in the necessary amount of water and then adding the glucose or other buffering agent thereto. If the diazo component is to be 30 applied simultaneously with the coupling component, as is conveniently the case when dyeing cellulose ester materials, it may be dispersed with the aid of Turkey red oil or other dispersing agent and mixed with the solution of the coupling 35 component. After the impregnation of the material with the coupling component, the materials are subsequently treated with a solution of the diazo compound of the diazo component, or, where the diazo and coupling components have 40 been applied to the materials, the latter may be treated so as to effect diazotization and coupling. In the case of a cellulose ester material impregnated with both diazo and coupling components, the material may be treated with an acidified 45 nitrite solution until diazotization is complete and thereafter subjected to a hot soaping treatment in order to complete the coupling.

A wide range of enolic coupling components may be applied to textile materials by the new 50 process. The latter is, however, of particular advantage in connection with the application of coupling components which are difficult to obtain in the form of true or colloidal solutions. Examples of such components are the arylamides 55 of 2:3- and other oxynaphthoic acids and arylamides of other hydroxy carboxylic acids, for example those of the benzene or carbazole series. Again, the invention is of value in connection with the application of  $\beta$ -keto acidyl derivatives 60 of aromatic amines and especially the di- $\beta$ -keto acidyl derivatives of aromatic diamines, as exemplified for instance by the diaceto-acetyl derivative of ortho-tolidine, commonly known as naphthol AS/G. Still other coupling components 65 may, however, be applied by the new process, for example  $\beta$ -naphthol, or coupling components generally containing hydroxyl and acidylamino groups, for example the 2-acidylamino-3-naphthols or the 1-acidylamino-7-naphthols. 70

In the case of cellulose ester or ether materials, the absorption of the enolic coupling components and/or any diazo component applied simultaneously therewith, may be facilitated by incorporating swelling agents in the baths, padding 75

liquors or printing pastes employed, or if desired the materials may be pretreated with swelling agents. Alcohol is a particularly suitable agent for this purpose, though other swelling agents may be employed, if desired.

As indicated previously, the invention is of special value in connection with the colouration of cellulose acetate or other cellulose ester materials. As examples of such materials mention 10 may be made, in addition to cellulose acetate, of cellulose formate, propionate or butyrate or mixed esters of cellulose, for example cellulose acetate-butyrate or nitroacetate or materials obtainable by treating cellulose with esterifying 15 agents, while retaining its fibrous form, for example the products obtainable by treating alkali cellulose with paratoluene sulphonic chloride, benzoyl chloride or other acid halides. Other materials may, however, also be coloured by the new 20 process, for example ethyl or benzyl cellulose or other cellulose ethers. Again, animal fibres are advantageously coloured by the new method, for example wool or natural silk, or, if desired, mixed materials containing for instance one or more of 25 the foregoing esters or ethers of cellulose or an animal fibre in conjunction with cotton, regenerated cellulose or other cellulosic fibre. In general, in the case of such a mixed material, the cellulosic component will be left substantially 30 uncoloured under the conditions of alkalinity most suitable for effecting the coloration of a cellulose ester or an animal fibre.

The following examples illustrate the invention but it is to be understood that they do not 35 limit it in any way:—

#### EXAMPLE 1

*To dye a deep crimson shade, fast to washing, on 10 kilos of yarn*

40 100 grams of 5-nitro-2-aminoanisole are dispersed by heating with 300 grams of Turkey red oil. 200 grams of 2'-oxy-3'-naphthoyl- $\beta$ -naphthylamine are dissolved with 400 grams of Turkey red oil and 50 grams of caustic soda in about 10 litres of hot water. To this is added a solution of 100 grams of glucose and the whole of these 45 solutions sieved into a dyebath of 300 litres set at 30° C. The previously well scoured yarn is entered, turned for  $\frac{1}{4}$  hour, and the temperature slowly raised over  $\frac{1}{2}$  an hour to 70° C. and kept 50 at this for one hour further. The yarn is then lifted and rinsed, and diazotized by working for  $\frac{1}{2}$  an hour in a cold bath prepared with 4 grams of sodium nitrite and 8 grams of glacial acetic acid per litre. The yarn is again lifted and rinsed, and turned for a  $\frac{1}{4}$  hour in a cold bath containing  $\frac{1}{2}$  gram per litre soda ash, lifted and entered into a bath containing 1 gram per litre good textile soap, and turned cold for  $\frac{1}{4}$  hour. The 55 temperature is then slowly raised to 75° C. and the yarn turned at this temperature until the correct shade is obtained, then lifted, rinsed, and dried or otherwise treated as requisite.

#### EXAMPLE 2

*To dye a full lemon-yellow shade on 10 kilos of cellulose acetate knit fabric*

70 100 grams of 2:5 dichloraniline, 125 grams of diacetooacetyl-orthotolidine, 100 grams caustic soda, and 500 grams of Turkey red oil, are heated together until a clear dispersion is obtained. This is filtered into a dyebath of 300 litres of

soft water at 50° C. in which 400 grams of corn syrup has previously been dissolved. The scoured fabric is entered and worked for  $\frac{1}{2}$  an hour at 50° C. and the temperature gradually raised to 75° C. and kept at this for an hour. The 5 bath is then dropped, and the fabric rinsed off, and diazotized by working for  $\frac{1}{2}$  an hour cold in a fresh bath prepared with 4 grams per litre sodium nitrite and 5 ccs. per litre formic acid. The diazotization bath is dropped, and the fabric 10 thoroughly rinsed, and soaped up to shade and finished as in Example 1 above.

#### EXAMPLE 3

*To dye a fast blue shade on 10 kilos of natural silk yarn*

200 grams of 2'-oxy-3'-naphthoyl-ortho-toluidine, 50 grams of caustic soda and 200 grams of Turkey red oil are heated with 10 litres of water until 20 solution is complete. This solution is then filtered into a dyebath of 300 litres of soft water at 50° C. containing 150 grams of glucose and the silk yarn entered and turned for  $\frac{1}{2}$  an hour at this temperature, and the temperature then 25 gradually raised over a further  $\frac{1}{2}$  an hour to 95° C. and kept at this for a further hour. The 30 yarn is then cooled off in the bath to 50° C. and then rinsed and entered into coupling bath at 70° C. containing a sufficiency of the diazo compound from 4'-methoxy-4-aminodiphenylamine and also a suitable protective colloid. When coupling is complete, the yarn is lifted, thoroughly rinsed, and soaped to shade at 95-98° C. then again lifted, rinsed, and dried, or otherwise treated 35 as requisite.

#### EXAMPLE 4

*To dye 10 kilos of a cotton/cellulose acetate woven fabric a fast blue shade on the cotton and a fast golden brown shade on the cellulose acetate* 40

The cotton is first dyed in a suitable machine with Indanthrene Blue 5G (Colour Index No. 1111) under conditions which do not affect the 45 cellulose acetate, and well washed off.

120 grams of the anilide of 2-oxycarbazole-3-carboxylic acid, 50 grams of paranitroaniline, 50 grams of caustic soda and 250 grams of Turkey red oil are dispersed by heating with sufficient 50 water and filtered into a dyebath of suitable volume at 50° C. To this is added a solution of 150 grams of invert sugar, and dyeing begun. The temperature is gradually raised to 75-80° C. and kept at this for 2-3 hours. The fabric is then 55 rinsed, and diazotized at 30° C. for  $\frac{1}{2}$  an hour in a bath prepared with 5 grams per litre sodium nitrite and 10 ccs. per litre glacial acetic acid. The fabric is again rinsed and soaped at 75° C. for  $\frac{1}{2}$  an hour, rinsed and dried or otherwise 60 treated as desired.

What we claim and desire to secure by Letters Patent is:—

Process for impregnating cellulose acetate materials with a diazotizable amine and an enolic coupling component, which comprises immersing the materials in an aqueous bath containing a diazotizable amine and the constituents of a composition obtainable by adding a reducing sugar to a solution of an enolic coupling component in 65 70 aqueous caustic alkali.

ERNEST WILLIAM KIRK  
GEORGE HOLLAND ELLIS.